# EUROPEAN PATENT SPECIFICATION

(11) **EP 1 037 723 B1**
(45) Date of publication and mention of the grant of the patent: **26.03.2003**
(21) Application number: 98954659.3
(22) Date of filing: 27.11.1998
(51) Int. Cl.: B22C 7/02, B22C 9/04

(54) **METHOD OF FORMING A CERAMIC MOLD**
VERFAHREN ZUR HERSTELLUNG VON KERAMIKFORMEN
PROCEDE POUR FORMER DES MOULES CERAMIQUE

(30) Priority: 08.12.1997 US 986861
(43) Date of publication of application: 27.09.2000
(73) Proprietor: Milwaukee School of Engineering, Milwaukee, WI 53202 (US)
(72) Inventor: TOBIN, James Robert, Charlotte NC 28277 (US)
(74) Representative: Grünecker, Kinkeldey, Stockmair & Schwanhäusser Anwaltssozietät
(86) International application number: IB9801887
(87) International publication number: WO99029451

(56) References cited:
- EP-A- 0 240 190
- EP-A- 0 625 386
- US-A- 4 617 977
- US-A- 5 507 336
- PATENT ABSTRACTS OF JAPAN vol. 007, no. 173 (M-232), 30 July 1983 & JP 58 077740 A (MITSUBISHI JUKOGYO KK), 11 May 1983

## Description

This invention relates to a method for preparing an accurate ceramic mold which can be used to create a more durable metal mold for casting multiple plastic parts similar to an original pattern.

Getting new products to the market faster than one's competition is recognized as a key to gaining a large market share. One area of product development having a significant impact on overall market timing is the making of product and package prototypes for market testing. Such testing usually requires multiple look-like, feel-like, and function-like prototypes for consumers to examine or use.

Package components generally involve plastic parts made in very expensive, multiple cavity, steel molds. For example, most bottles are blow-molded and most bottle closures are injection molded. It usually takes large production quantities to justify the cost of a production mold with many cavities. For smaller markets, or for making only a few hundred test parts, single cavity molds or prototype molds are created. Prototype molds provide important learning on whether the part can be made consistently, as well as to provide a tool that can be used to make test parts. In the case of making molds from production class metals such as P20 or H13 steel, often electro discharge machining (EDM) is used. EDM electrodes are shaped to generate reverse patterns in the metal they are applied to. Such electrodes are typically machined from copper or graphite. These electrode materials break down and wear in the EDM process and replacement electrodes must be machined and substituted in order to complete the EDM process. Increased wear resistance materials for EDM electrodes are now available, but they cannot be easily machined. What is needed is a method of making high wear resistant electrodes without having to machine them.

One method of rapidly prototyping containers or parts is investment casting using patterns generated by rapid prototyping systems instead of traditional injection molded wax patterns. An example of such a pattern is a QUICKCAS™ pattern, a Trademark of 3D Systems, Inc. of Valencia, CA. A hollow plastic pattern is coated with a thin ceramic shell usually by a dipping process. The plastic is burned out of the ceramic shell leaving minimal amounts of ash residue behind. Molten metal is then poured into the ceramic shell to cast a metal part or metal mold for a plastic part. Because the shell has only a small hole for admitting molten metal, it is difficult to inspect the critical surfaces for ash residue. Any ash residue on a critical surface will potentially ruin the metal casting. The molten metal cools and shrinks such that critical surfaces are not reproduced accurately. The larger the parts, the greater the inaccuracy.

An example of an investment casting process where a lost pattern is formed in a lost mold is known from EP 625 386 A1.

An improved method of constructing a fully dense mold is disclosed in U.S. 5,507,336 issued to Tobin, April, 1996. The method comprises placing a pattern within a tube which has a melting point greater than that of the infiltration material which will be used in making the metal mold. A ceramic member is cast between the pattern surfaces and the open end of the tube to transfer the critical pattern surfaces to the ceramic member. The ceramic surfaces are inverse to the pattern surfaces. The pattern is burned out and the ceramic surfaces remains in the tube. The ceramic is then covered with metal powder and an infiltration material from the other end of the tube, and the tube is placed in a furnace to form the metal part over the ceramic surfaces. The metal part has surfaces inverse to the ceramic surfaces. A metal mold results when the ceramic piece is removed. The metal mold has the same shape as the pattern, and is useful for molding plastic parts having an inverse shape. This is an ideal process for parts having exterior critical surfaces.

Tobin's process destroys the pattern from which the ceramic mold is created. A process for quickly forming a ceramic mold pattern which does not destroy the pattern, but which is accurate, is needed. Also, it is often necessary to provide a mating metal mold for plastic part molding. In order to do this, the metal mold may require a shape which is the inverse of the pattern. Thus, the ceramic mold needs to have the same shape as the pattern, and therefore requires an intermediate mold be produced between the ceramic mold and the pattern. As with Tobin's earlier process, any ceramic mold should not be contaminated on its surface so that the resulting metal mold is accurate.

In order to avoid destroying the pattern, it is desirable to use an intermediate mold made of a material which can be discarded or reused as needed to transfer the critical pattern surfaces to the ceramic mold. Wax and silicone rubbers have been used for these purposes. Wax (which is heat reversible) has the disadvantage of being brittle and when removed from the pattern can cause small pieces to break off especially where undercuts and thin features are involved. It also can expand and crack the ceramic when heated. Silicone rubbers need to be cured, and when the ceramic releases heat as it "sets", the silicone rubber can distort and cause inaccuracies to develop in the ceramic pattern. Also, silicone rubber has to be removed from the pattern by air injection or other means which forces the silicone from the ceramic. This can cause the ceramic mold to break especially where thin features are involved.

It is therefore an object of the present invention to provide a process for making a ceramic mold having the same shape as a pattern, which produces accurate reproductions of a pattern of any size, within a tolerance of ±0.005 inches and which does not leave an ash or other residue on the ceramic mold.

Said object is achieved according to the invention by a method having the features of claim 1 and a method having the features of claim 4. Preferred embodiments of the invention are defined in the sub-claims.

The present invention will now be explained in detail by the following description of preferred embodiments, taken in conjunction with the accompanying drawings, in which like reference numeral identify identical elements and wherein:
Figure 1 is a sectioned front elevational view of a pattern **1**, having critical pattern surfaces **13**, positioned inside a first flask **3**.
Figure 2 is a sectioned front elevational view of pattern **1** inside the first flask **3** into which a liquid metal **5** has been poured.
Figure 3 is a sectioned front elevational view of a solidified metal mold **7**, having critical metal mold surfaces **10** transferred from critical pattern surfaces **13**, positioned inside a second flask **8** with an annular space **12** between second flask **8** and solidified metal mold **7**.
Figure 4 is a sectioned front elevational view of second flask **8** having a plaster or ceramic solution **9** poured over the solidified metal mold **7** and into annular space **12** and covering critical metal mold surfaces **10**.
Figure 5 is a sectioned front elevational view of a solidified plaster mold **11** from which has been removed second flask **8** and metal mold **7**, exposing critical ceramic surfaces **14**, which transferred from critical metal mold surfaces **10** and which accurately replicate critical pattern surfaces **13.**

### DETAILED DESCRIPTION OF THE INVENTION

As used herein, the term "ceramic" refers to a material such as plaster, clay, silica or other nonmetallic material which can be fired to create a hardened product.

As used herein, the term "metal" refers to any metal, metal alloy, or metal alloy composite that melts below a temperature at which damage to a pattern may occur, or which could cause substantial thermal expansion of the pattern. This metal, metal alloy, or metal alloy composite does not substantially expand or shrink upon solidification. It also freezes above a temperature that could cause substantial thermal contraction of the pattern. Preferably, it solidifies at about 3° C above room temperature. The metal forms a solid which has minimal expansion or shrinkage when exposed to a range of temperatures associated with pouring a ceramic that sets into a solid shape.

As used herein, the term "heat reversible" refers to a metal which solidifies at a temperature below about 35°C and which melts or liquifies at temperatures above about 45°C. Although there are non-metal thermally reversible materials available, such as gelatins, a low melting point metal is believed fastest to melt because of its high thermal conductivity. Also, a low melting point metal has a lower viscosity than gelatin doesn't have a s much tendency to wash away ceramic surface particles when removed from a ceramic mold. Such fine ceramic particles are key to maintaining a good surface finish of parts cast therefrom.

Figure 1 illustrates a pattern **1** which fits tightly against an internal surface of a first flask. Pattern 1 is a representation of the exterior of a bottle closure. Pattern 1 has critical pattern surfaces, **13**, which represent the detail on the outside of the bottle closure. The pattern is preferably made by a stereolithography process, well known in the prototyping art, in which an electronic file describing the pattern is rapidly fabricated by laser curing of a polymer. The pattern (1) is placed in the first flask (3) with critical pattern surfaces (13) facing upward toward the open end of the first flask.

A liquid metal (5) is poured over the pattern (1). The metal mold (7) is intended to be an intermediate mold which transfers the critical pattern surfaces (13) to a ceramic mold (11). A ceramic solution (9) is similarly poured over the metal mold (7) in an open second flask (8) and allowed to harden. However, the ceramic material typically generates heat in an exothermic binding reaction. The metal mold (7) must eventually be removed from the ceramic mold (11) by melting the metal. Where there are thin sections melting the metal away avoids damage to the brittle ceramic mold (11). The reliquified metal is easily removed from a ceramic mold (11) by pouring it out. The exothermic reaction of the ceramic typically melts the metal adjacent to it so that surface distortions do not occur as the ceramic hardens. The resulting ceramic mold (11) can be washed with molten brazing flux to remove any residue before firing the ceramic mold (11) to harden it.

The preferred metal is CERROLOW® 117, a Trademark of Cerro Corporation, and is available from Cerro Metal Products of Bellefonte, PA. Fibers or other structural materials can be dispersed in the metal. These will add strength and can be easily removed with the melted metal from the ceramic mold (11).

The metal is poured over the pattern (1) in an open ended flask, as shown in Figure 2. The metal casting may be done in multiple pours, depending on the size of the part. The first pour of a multiple pour is preferably allowed to form a skin before the next pour so that air bubbles will not penetrate the first pour.

The first flask is refrigerated or allowed to cool in ambient room temperature until the metal has solidified. Depending on the size of the pattern (1), and the depth of the metal layer, from about 2 to about 8 hours are required to solidify the metal.

The depth of the metal pour will depend upon the pattern (1) and the size that is desired for the ceramic mold (11). One skilled in the art can easily determine this without undue experimentation. Typically, a minimum metal thickness of about 2.5 cm is desired above each critical pattern surface (13).

The solidified intermediate metal mold (7) is then pulled from the pattern (1). In a preferred embodiment, the first flask is built with easily removable sides which are then pulled off the metal mold (7) and the metal mold (7) is then pulled off the pattern (1). The metal mold (7) retains the inverse replications of the critical surfaces (13) of the pattern (1) without distortion, even when thin features are involved. It is important that the pattern (1) have smooth surfaces with no undercuts. Undercuts and rough surfaces can prohibit removal of the solidified metal from the pattern (1).

Figure 3 discloses the metal mold (7) placed in a second flask (8) to which a plaster or ceramic solution (9) will be added. The metal mold (7) is placed with the critical metal mold surfaces (10) facing upward toward the open end of the second flask (8). Preferably, sufficient space (12) is allowed between the second flask (8) and the metal mold (7) so that ceramic will be formed around the metal mold (7) in that space (12). The ceramic mold (11) made therefrom will have a continuous annular ceramic rim surrounding the critical ceramic surfaces (14) so that the ceramic mold (11) may be readily used for casting purposes without the need for another flask.

Plaster or other ceramic material (3) is poured into the second flask (8) to a depth above the metal mold (7). Preferably, the depth is from about 1 cm to about 5 cm above the metal mold (7). The poured ceramic material (4) is preferably degassed under vacuum to remove any air which could affect the final ceramic mold formation. The plaster or ceramic material first "sets" or takes a solid shape and then completely solidifies. During the binding process, an exothermic reaction takes place in the plaster which melts the surrounding metal. The second flask (8) is preferably coated with a release agent so that the second flask (8) may be easily removed from the ceramic mold (11).

The preferred exothermic ceramic material is C1-Core Mix, available from Ranson & Randolph of Maumee, Ohio. It is a mixture of fused silica, zirconium silicate, ammonium phosphate, silica (cristobalitc) and magnesium oxide. Core hardener 2000, also available from Ranson & Randolph, can be used. It contains amorphous silica and dipotassium-6-hydroxy -3- oxo -9- xanthene -0- benzoate.

After the ceramic is set, the ceramic mold (11) and remaining metal can be heated in an oven or by a heat gun to completely melt the metal for easy removal. The temperature of the oven should be about 200°C to about 500°C to insure the melting of the metal.

The open end of the ceramic mold (11), which corresponds to the bottom end of the second flask (8), allows easy access to pour the melted or liquid metal from the ceramic mold (11). Also, critical ceramic surfaces (14) may be easily inspected from the open end to see that all metal and any residue are removed.

Placing the ceramic mold (11) in a furnace and heating it to at least 1100°F (990°C) for at least 3 hours fully sets the plaster for further processing. A hydrogen atmosphere can be used as there is no residue remaining on the ceramic which needs to be burned off. This lack of residue is an important distinction when compared to ceramic mold making processes using epoxies and waxes.

## Claims

1. A method for forming a ceramic mold comprising the steps of:
a) placing a pattern (1) having critical pattern surfaces (13) in a first flask (3) having an open end, said pattern surfaces (13) facing upward toward said open end;
b) covering said critical pattern surfaces (13) with a heat reversible liquid metal (5) added to said first flask (3) and;
c) cooling said liquid metal (5) while degassing said liquid metal (5) to form a solid metal mold (7), said metal mold (7) having critical metal mold surfaces (10) transferred from said critical pattern surfaces (13) which are inverse to said critical pattern surfaces (13);
d) removing said pattern (1) and said first flask (3) from said metal mold (7) and placing said metal mold (7) in a second flask (8) with said critical metal mold surfaces facing upward toward an open end of said second flask (8);
e) covering said critical metal mold surfaces (10) with a ceramic solution (9) added to said second flask (8) while degassing said ceramic solution (8), said ceramic solution (9) solidifying and then exothermically binding to form a ceramic mold (11) around said metal mold (7), said ceramic mold (11) having critical ceramic surfaces (14) transferred from said critical metal mold surfaces (10) which are inverse to said critical metal mold surfaces (10), said ceramic critical surfaces (14) thereby accurately replicating said critical pattern surfaces (13); and
f) liquifying said metal mold (7) via heating to remove said metal from said ceramic mold (11) and removing said second flask (8) from said ceramic mold (11).

2. The method according to claim 1, further **characterized in that** said metal is CERROLOW® 117.

3. The method according to claim 1, further **characterized in that** said liquid metal (5) further comprises fibers or other thickeners.

4. A method for forming a ceramic mold comprising the steps of:
a) placing a pattern (1) having critical pattern surfaces (13) in a first flask (3) having an open end, said critical pattern surfaces (13) facing upward toward said open end;
b) covering said critical pattern surfaces (13) with a metal solution (5) added to said first flask (8) and;
c) cooling said metal solution (5) while degassing said metal solution (5) to form a solid metal mold (7), said metal mold (7) having critical metal mold surfaces (10) transferred from said critical pattern surfaces (13) which are inverse to said critical pattern surfaces (13);
d) removing said pattern (1) and said first flask (3) from said metal mold (7) and placing said metal mold (7) in a second flask (8) with said critical metal mold surfaces (10) facing upward toward an open end of said second flask (8), said second flask (8) dimensioned to provide an annular space (12) around said metal mold (7);
e) filling said annular space (12) with a first ceramic solution added to said second flask (8) while degassing said first ceramic solution, said first ceramic solution solidifying without generating heat to form a first ceramic mold in order to anchor said metal mold (7) in place and to form a continuous annular rim surrounding said critical metal mold surfaces;
f) covering said first ceramic mold and said metal mold with a second ceramic solution added to said second flask (8), said second ceramic solution exothermically binding to form a second ceramic mold bonded to said first ceramic mold, said second ceramic mold having critical ceramic surfaces transferred from said critical metal mold surfaces (10) which are inverse to said critical metal mold surfaces (10), said critical ceramic surfaces thereby accurately replicating said critical pattern surfaces (13); and
g) liquifying said metal mold (7) via heating to remove said metal from said first and second ceramic molds and removing said second flask (8) from said first and second ceramic molds.

## Patentansprüche

1. Verfahren zum Herstellen einer Keramikform, aufweisend die Schritte:
a) Platzieren eines Musters (1), das kritische Muster-Oberflächen (13) besitzt, in einen ersten Kasten (3), der ein offenes Ende besitzt, wobei die Muster-Oberflächen (13) nach oben zu dem offenen Ende hinweisen;
b) Abdecken der kritischen Muster-Oberflächen (13) mit einem wärme-reversiblen, flüssigen Metall (5), hinzugegeben zu dem ersten Kasten (3), und
c) Kühlen des flüssigen Metalls (5), während das flüssige Metall (5) entgast wird, um eine feste Metallform (7) zu bilden, wobei die Metallform (7) kritische Metallform-Oberflächen (10) besitzt, die von den kritischen Muster-Oberflächen (13) übertragen sind, die invers zu den kritischen Muster-Oberflächen (13) sind;
d) Entfernen des Musters (1) und des ersten Kastens (3) von der Metallform (7) und Platzieren der Metallform (7) in einen zweiten Kasten (8) mit den kritischen Metallform-Oberflächen nach oben zu einem offenen Ende des zweiten Kastens (8) hinweisend;
e) Abdecken der kritischen Metallform-Oberflächen (10) mit einer keramischen Lösung (9), hinzugefügt zu dem zweiten Kasten (8), während die keramische Lösung (8) entgast wird, wobei die keramische Lösung (9) verfestigt wird und dann exotherm gebunden wird, um eine keramische Form (11) um die Metallform (7) herum zu bilden, wobei die Keramikform (11) kritische, keramische Oberflächen (14) besitzt, übertragen von den kritischen Metallform-Oberflächen (10), die invers zu den kritischen Metallform-Oberflächen (10) sind, wobei die keramischen, kritischen Oberflächen (14) dadurch akkurat die kritischen Muster-Oberflächen (13) replizieren; und
f) Verflüssigen der Metallform (7) über Erwärmung, um die Metallform von der Keramikform (11) zu entfernen und den zweiten Kasten (8) von der Keramikform (11) zu entfernen.

2. Verfahren nach Anspruch 1, das weiterhin **dadurch gekennzeichnet ist, dass** das Metall CERROLOW® 117 ist.

3. Verfahren nach Anspruch 1, **dadurch gekennzeichnet, dass** das flüssige Metall (5) weiterhin Fasern oder andere Verdickungsmittel aufweist.

4. Verfahren zum Bilden einer Keramikform, aufweisend die Schritte:
a) Platzieren eines Musters (1), das kritische Muster-Oberflächen (13) besitzt, in einen ersten Kasten (3), der ein offenes Ende besitzt, wobei die kritischen Muster-Oberflächen (13) nach oben zu dem offenen Ende hinweisen;
b) Abdecken der kritischen Muster-Oberflächen (13) mit einer Metalllösung (5), hinzugefügt zu dem ersten Kasten (3), und
c) Kühlen der Metalllösung (5), während die Metalllösung (5) entgast wird, um eine feste Metallform (7) zu bilden, wobei die Metallform (7) kritische Metallform-Oberflächen (10) besitzt, die von den kritischen Muster-Oberflächen (13) übertragen sind, die invers zu den kritischen Muster-Oberflächen (13) sind;
d) Entfernen des Musters (1) und des ersten Kastens (3) von der Metallform (7) und Platzieren der Metallform (7) in einen zweiten Kasten (8) mit den kritischen Metallform-Oberflächen (10) nach oben zu einem offenen Ende des zweiten Kastens (8) hinweisend, wobei der zweite Kasten (8) so dimensioniert ist, um einen ringförmigen Raum (12) um die Metallform (7) herum zu schaffen;
e) Füllen des ringförmigen Raums (12) mit einer ersten, keramischen Lösung, hinzugefügt zu dem zweiten Kasten (8), während die erste, keramische Lösung entgast wird, wobei die erste, keramische Lösung ohne Erzeugen von Wärme verfestigt wird, um eine erste Keramikform zu bilden, um die Metallform (7) an ihrer Stelle zu verankern und um einen kontinuierlichen, ringförmigen Rand zu bilden, der die kritischen Metallform-Oberflächen umgibt;
f) Abdecken der ersten keramischen Form und der Metallform mit einer zweiten, keramischen Lösung, hinzugefügt zudem zweiten Kasten (8), wobei die zweite, keramische Lösung exotherm bindet, um eine zweite Keramikform, angebunden an der ersten Keramikform, zu bilden, wobei die zweite Keramikform kritische, keramische Oberflächen besitzt, übertragen von den kritischen Metallform-Oberflächen (10), die invers zu den kritischen Metallform-Oberflächen (10) sind, wobei die kritischen, keramischen Oberflächen dadurch akkurat die kritischen Muster-Oberflächen (13) replizieren; und
g) Verflüssigen der Metallform (7) über Erwärmung, um das Metall von der ersten und der zweiten Keramikform zu entfernen, und Entfernen des zweiten Kastens (8) von der ersten und der zweiten Keramikform.

## Revendications

1. Procédé pour former un moule en céramique, comprenant les étapes consistant à :
a) placer un motif (1) ayant des surfaces de motif (13) critiques dans un premier châssis (3) ayant une extrémité ouverte, lesdites surfaces de motif (13) étant tournées vers le haut en direction de ladite extrémité ouverte ;
b) couvrir lesdites surfaces de motifs (13) critiques avec un métal (5) se liquéfiant de façon réversible sous l'effet de la chaleur, ayant été ajouté audit premier châssis (3) et ;
c) refroidir ledit métal liquide (5) tout en dégazant ledit métal liquide (5) pour former un moule métallique (7) solide, ledit moule métallique (7) ayant des surfaces de moule (10) métalliques critiques, transférées depuis lesdites surfaces de motif (13) critiques qui sont l'inverse desdites surfaces de motif (13) critiques ;
d) enlever ledit motif (1) et dudit premier châssis (3) dudit moule métallique (7) et placement dudit moule métallique (7) dans un deuxième châssis (8), lesdites surfaces de moule en métal critique étant tournées vers le haut, en direction d'une extrémité ouverte dudit deuxième châssis (8) ;
e) couvrir lesdites surfaces de moule (10) métalliques critiques par une solution céramique (9) ajoutée audit deuxième châssis (8) tout en dégazant ladite solution céramique (8), ladite solution céramique (9) se solidifiant puis subissant un phénomène de prise exothermique pour former un moule céramique (11) autour dudit moule métallique (7), ledit moule métallique (11) ayant des surfaces céramiques (14) critiques, transférées depuis lesdites surfaces de moule (10) métalliques critiques qui sont l'inverse desdites surfaces de moule (10) métalliques critiques, lesdites surfaces céramiques (14) critiques de cette manière étant des répliques précises desdites surfaces de motif (13) critiques ; et
f) liquéfier ledit moule métallique (7) par un processus de chauffage pour enlever ledit métal dudit moule céramique (11) et enlever ledit deuxième châssis (8) dudit moule céramique (11).

2. Procédé selon la revendication 1, **caractérisé en outre en ce que** ledit métal est du CERROLOW® 117.

3. Procédé selon la revendication 1, **caractérisé en outre en ce que** ledit métal liquide (5) comprend en outre des fibres ou bien d'autres épaississants.

4. Procédé de formation d'un moule métallique comprenant les étapes consistant à :
a) placer un motif (1) ayant des surfaces de motif (13) critiques dans un premier châssis (3) ayant une extrémité ouverte, lesdites surfaces de motif (13) étant tournées vers le haut en direction de ladite extrémité ouverte ;
b) couvrir lesdites surfaces de motifs (13) critiques avec un métal (5) se liquéfiant de façon réversible sous l'effet de la chaleur, ayant été ajouté audit premier châssis (3) et ;
c) refroidir ledit métal liquide (5) tout en dégazant ledit métal liquide (5) pour former un moule métallique (7) solide, ledit moule métallique (7) ayant des surfaces de moule (10) métalliques critiques, transférées depuis lesdites surfaces de motif (13) critiques qui sont l'inverse desdites surfaces de motif (13) critique ;
d) enlever ledit motif (1) et dudit premier châssis (3) dudit moule métallique (7) et placement dudit moule métallique (7) dans un deuxième châssis (8), lesdites surfaces de moule en métal critique étant tournées vers le haut en direction d'une extrémité ouverte dudit deuxième châssis (8), ledit deuxième châssis (8) étant dimensionné pour fournir un espace annulaire (12) autour dudit moule métallique (7) ;
e) remplir ledit espace annulaire (12) avec une première solution céramique ajoutée audit deuxième châssis (8) tout en dégazant ladite première solution céramique, ladite première solution céramique (9) se solidifiant sans générer de chaleur, afin de former un premier moule céramique de manière, à ancrer ledit moule métallique (7) en place et à former une bordure annulaire continue entourant lesdites surfaces de moule métalliques critiques ;
f) couvrir ledit premier moule céramique et ledit moule métallique avec une deuxième solution céramique ajoutée audit deuxième châssis (8), ladite solution céramique se solidifiant en subissant un phénomène de prise exothermique pour former un deuxième moule céramique lié audit premier moule céramique, ledit deuxième moule céramique ayant des surfaces céramiques critiques, transférées depuis lesdites surfaces de moule (10) métalliques critiques, qui sont l'inverse desdites surfaces de moule (10) métalliques critiques, lesdites surfaces céramiques (14) critiques de cette manière étant des répliques précises desdites surfaces de motif (13) critiques ; et
g) liquéfier ledit moule métallique (7) par un processus de chauffage pour enlever lesdits premier et deuxième moules céramiques et enlever ledit deuxième châssis (8) dudit moule céramique (11).
